

No. 863,733.

PATENTED AUG. 20, 1907.

A. J. LUSTIG,

## PROCESS OR METHOD OF CASTING INGOTS.

APPLICATION FILED FEB. 1, 1900.

2 SHEETS-SHEET 1.



FIG. 2

FIG. 3



13



FIG. 4

**WITNESSES:**

Mrs. D. Richards  
Mary Ormsdell

FIG. 6

FIG. 5

**INVENTOR:**

**ADOLPHUS J. LUSTIG**

BY a7

BY  
Fred L. Fraenzel,  
ATTORNEY

No. 863,733.

PATENTED AUG. 20, 1907.

A. J. LUSTIG.

PROCESS OR METHOD OF CASTING INGOTS.

APPLICATION FILED FEB. 1, 1900.

2 SHEETS—SHEET 2.



WITNESSES:

Geo. D. Richards

Marcy J. Drewell

INVENTOR:

ADOLPHUS J. LUSTIG

BY  
FRED L. FRAENZEL  
ATTORNEY

# UNITED STATES PATENT OFFICE.

ADOLPHUS J. LUSTIG, OF NEWARK, NEW JERSEY, ASSIGNOR OF ONE-FIFTH TO ISAAC LEHMAN, OF NEWARK, NEW JERSEY, AND ONE-FIFTH TO LOUIS KAHN, OF NEW YORK, N. Y.

## PROCESS OR METHOD OF CASTING INGOTS.

No. 863,733.

Specification of Letters Patent.

Patented Aug. 20, 1907.

Application filed February 1, 1900. Serial No. 3,620.

To all whom it may concern:

Be it known that I, ADOLPHUS J. LUSTIG, a citizen of the United States, residing at Newark, in the county of Essex and State of New Jersey, have invented certain new and useful Improvements in the Process or Method of Casting Ingots; and I do hereby declare the following to be a full, clear, and exact description of the invention, such as will enable others skilled in the art to which it appertains to make and use the same, reference being had to the accompanying drawings, and to letters of reference marked thereon, which form a part of this specification.

This invention relates to the casting of steel ingots, and the invention has for its principal object the novel process to be hereinafter described, which consists in pouring molten metal into a mold, supplying hydro-carbon gas underneath, outside of and adjacent to the mold bottom, transmitting the heat from the molten metal to said gas, and thereby causing the hydro-carbon gas to pass through the mold in a continuous and unlimited supply and to rise into the molten metal in the mold especially during the time of pouring the molten steel into the mold; and, a further object of this invention is, in addition to this step above set forth, to also supply hydro-carbon gas to the upper portion of the mold, transmit heat from the molten metal in the mold to said gas, and thereby cause the hydro-carbon gas to pass into the upper portion of the mold and into the molten metal therein.

My novel method is preferably carried out by placing the open-bottomed mold upon a porous plate of metal which rests upon a hollow base into which the reducing gas, as hydro-carbon gas, is introduced so that the heat transmitted from the molten mass in the mold to the said porous plate of metal will distend or open the pores of such plate, and that the hydro-carbon gas will enter through the said pores in a continuous and unlimited supply into the molten metal contained in the mold, the gas acting as a re-agent upon the oxygen, nitrogen, and sulfur contained in the steel and also preventing all further admission of oxygen, nitrogen and humidity contained in the air into the said molten mass of steel while the solid ingot is being formed.

My invention therefore consists, primarily, in the several novel steps in the process or method of casting steel ingots, substantially as hereinafter more fully set forth, and then finally embodied in the clauses of the claims, which form a part of this specification.

This invention has for its further object, the novel process hereinafter described, which consists in pouring molten steel into a mold, arranged upon a hollow base or support, supplying the base or support with hydrogen or hydro-carbon gas, transmitting heat from the molten steel in the mold to said hollow base and said

gas, and passing the gaseous resultant into and through the molten steel in the mold.

In the accompanying drawings, I have illustrated one of the several forms of molds and mold-supports, employed with my novel process or method of casting ingots.

In the said drawings, Figure 1 is a vertical section of a mold-support, with the mold in position thereon, said mold being represented partly in vertical section and partly in elevation, and Figs. 2, 3, 4 and 5, are horizontal sections taken, respectively on line 2-2, 3-3, 4-4, and 5-5 in Fig. 1, to more clearly illustrate the inner arrangement of the mold-support, employed with my novel process or method of casting ingots. Fig. 6 is a vertical cross-section of the mold-support, taken on line 6-6 in Fig. 4. Fig. 7 is in part a side view of the bottom and a central vertical section of the upper portion of the ingot mold, said view also illustrating in side elevation the support for the mold, and a central vertical section of an oil-reservoir or tank attached to one side of the mold, at or near the top thereof. Fig. 8 is a part side view and part vertical section of a portion of the mold and a vertical section of the oil-reservoir or tank, and a means of communication for the passage of the volatile carbonaceous gas from the tank into the mold being represented in elevation; and Fig. 9 is a face view of the upper portion of the mold, the oil reservoir or tank having been removed.

Similar letters of reference are employed in all of the said above described views to indicate corresponding parts.

In the said drawings, in Figs. 1 to 6 inclusive, *a* indicates the base or foundation, on which the mold is to be supported, the same consisting, essentially, of a base-plate *a'* and the upwardly extending and surrounding sides *a*<sup>2</sup>, thus forming a receptacle or box-like base or foundation. Resting upon the inclined edges *a*<sup>4</sup> of inwardly extending ribs *a*<sup>3</sup>, preferably formed integral with the inner sides *a*<sup>2</sup> and with the inner surface of the base-plate *a'*, is a support *b* for the mold *d*. The said support *b* is preferably made in the manner of a truncated pyramid, of four sides, its downwardly tapering sides *b*<sup>1</sup> resting upon said ribs *a*<sup>3</sup>, substantially as illustrated, whereby the surrounding open spaces *a*<sup>5</sup> are formed, as clearly illustrated in Fig. 5. The spaces are filled with a loose material *a*<sup>6</sup>, such as pumice stone, asbestos, or other material of a like nature.

Leading into and extending through one or more sides of the receptacle, or box-like foundation *a* are suitable gas-conveying pipes or other suitable ducts *a*<sup>7</sup>, which communicate with the passage-ways or ducts *a*<sup>13</sup> and *b*<sup>6</sup> and finally with a central duct or chamber *b*<sup>8</sup> in the support *b*, from the upper portion of which radiate or extend other ducts or passage-ways *b*<sup>2</sup> into

the open spaces  $a^5$ . These ducts  $b^2$  terminate, preferably, in front of the inclined edges of the ribs  $a^3$ , where the latter are cut away to form suitable passage-ways  $a^8$ , for the gas from said ducts  $b^2$  into the said spaces  $a^6$ . Of course, it will be understood, that the said ducts  $b^2$ ,  $b^6$  and  $a^{13}$ , however, may be arranged in any other suitable and practical manner, so as not to terminate directly in front of the said ribs.

- The upper surface of the mold-support  $b$  is preferably 10 provided with raised portions  $b^4$ , of any desirable configuration, and with channels  $b^3$  for reducing the metal at the upper part of the support, and for the accumulation of the volatile gas therein, for the purposes to be hereinafter fully set forth. Resting directly upon the 15 upper surface of this support  $b$  is a porous cast iron plate  $c$ , which is planed off on both sides, and is preferably provided with a square or other suitably shaped depression or recess  $c'$  in which is placed a metal plate  $c^2$ , and a plate or layer  $c^3$ , of refractory material, as 20 asbestos and fire-clay upon which the stream of molten metal is received when first poured into the mold  $d$  through the pouring opening  $a^6$  in the plate or cover  $d'$  resting upon the top of the mold. The mold  $d$  rests centrally upon said plate  $c$ , being surrounded by the 25 plates  $e$ , which consist, preferably, of four pieces, as shown in Figs. 2 and 3 of the drawing, and are provided with handles or other lifting means  $e'$  for the removal of said plates, when desired. Surrounding the outer and lower portion of the mold  $d$  and resting upon said 30 plates  $e$  is a vessel or hollow frame  $f$ , provided with perforations or holes  $f^2$  in its sides  $f'$  which surround the lower portion of the mold, said frame being for the reception of a carbonaceous material, such as asphaltum and mineral oil, or a compound containing 35 the same. The mold  $d$ , which may be of any well known form and of the usual material such as iron, or the like, is preferably recessed in its several sides, as at  $d^2$ , and has secured in said recesses, certain steel plates  $d^3$ , which are secured in position by means of 40 bolts  $d^4$  screwed into the mold and passing through slots  $d^5$  in said plates  $d^3$ , to allow of the expansion and contraction of said plates, as the mold becomes heated and cooled, also for the purpose of preventing undue outward radiation of the heat from within the mold, 45 said plates furthermore preventing the escape of the volatile hydro-carbon through the porous material of which the ingot mold is made. These several parts being in the positions indicated in Figs. 1 to 6 inclusive, hydro-carbon gas or hydrogen gas is slowly admitted through the pipe or pipes  $a^7$ , into the ducts  $a^{13}$  50 and  $b^6$ , the central passage-way  $b^8$  and through the ducts  $b^2$  into the open spaces  $a^6$  and the loose material  $a^6$  therein, the said hydro-carbon gas first expelling all atmospheric air from the foundation  $a$ , and passing 55 through the pores of the heated supporting plate  $c$ , which may be termed and in practice does form one of the walls of the mold, into the mold  $d$ , in which the hydro-carbon gas mixes with the fluid steel, as will be clearly evident.
- 60 Instead of introducing a hydrocarbon gas into the mold base, a quantity of a liquid hydrocarbon may be placed or stored therein, which will be gradually volatilized by the heat from the molten metal, thus supplying the hydrocarbon gas employed for treating the steel. At the same time, the heat from the molten metal is

transmitted to the frame  $f$ , and the carbonaceous material  $f^3$  in said frame  $f$  begins to melt and flows through the openings  $f^2$  in said frame  $f$  down the lower portions of the sides of the mold to the joint formed between the lower end-surface of the mold and the supporting 70 or base-plate  $c$  upon which the mold  $d$  rests. In this manner, the hydrogen gas or hydro-carbon gas from the box-like foundation  $a$  and the volatile gas from the liquid hydro-carbon, coming from the frame  $f$  is drawn or otherwise forced into the bottom of the mold  $d$  and 75 into the semi-fluid steel therein. At the same time, the liquid hydro-carbon from the frame  $f$  fills up the surrounding crevices, thereby preventing any influx of atmospheric air into the bottom of the mold, to prevent oxidation of the steel, and also effecting the 80 deoxidation of the fluid steel which has become oxidized while in transit from the ladle into the mold, as will be clearly evident. All oxygen is in this manner driven off with the hydro-carbon gas, and the metal is held in a proper condition free from oxids of carbon 85 which tend to reduce the value of the metal and are the cause of imperfect ingots. Furthermore, I may arrange upon one side of the mold  $d$ , at or near the top thereof a reservoir or tank  $l$ , see Fig. 1, which is provided with a nozzle  $l'$  for filling the tank with a liquid 90 hydro-carbon, the tank being supported upon the side by means of an eye  $l^2$  and hook  $l^3$ , or in any other manner, and having one or more ducts  $l^4$  which extend into the inner and upper portion of the mold  $d$ , each duct or pipe  $l^4$  being provided with a downwardly extending 95 nozzle  $l^5$ , substantially as illustrated. These pipes  $l^4$ , as will be seen from Figs. 7, 8 and 9 of the drawing, are removably placed in recesses  $d^6$  in the upper portion of the mold, which permits of the tank or reservoir  $l$  being removed from the side of the mold, when 100 the cover  $d'$  is taken off. The radiated heat from the cooling steel in the mold and that from the mold itself, will cause the carbonaceous oil in the tank  $l$  to give off a hydro-carbon gas which is admitted into the upper portion of the mold  $d$ . This gas is thus directed 105 directly to that portion of the semi-fluid mass in the mold where the "piping" in ingots occurs, and I prevent this "piping" or shrinkage of the ingot by then pouring from the ladle, a further quantity of molten steel in a semi-solid state into this upper portion of the 110 mold filled with the hydrocarbon gas from said tank or reservoir  $l$ , and I thereby avoid the "piping" of the ingot.

Having thus described my invention, what I claim is:

1. The process of casting ingots, which consists in introducing the molten metal into a mold, passing into and through said metal a continuous stream of a heated gas capable of removing therefrom oxygen, nitrogen and sulfur, and permitting the cast metal to cool, as set forth. 120
2. The process of casting ingots, which consists in introducing the molten metal into a mold, passing into and through said metal a continuous stream of a heated hydrocarbon gas, and permitting the cast metal to cool, as set forth. 125
3. The process of casting ingots, which consists in introducing the molten metal into a mold having a wall which is permeable to gas but not to molten metal, and forcing a purifying gas through said wall and into said metal, as set forth. 130
4. The process of casting ingots, which consists in introducing the molten metal into a mold having a wall which is permeable to gas but not to molten metal, and

forcing a deoxidizing gas through said wall and into said metal, as set forth.

5. The process of casting ingots, which consists in introducing the molten metal into a mold having a wall which is permeable to gas but not to molten metal, and forcing through said wall and into said metal a gas capable of removing oxygen, nitrogen and sulfur from said metal, as set forth.

6. The process of casting ingots, which consists in 10 introducing the molten metal into a mold having a wall which is permeable to gas but not to molten metal, and forcing a hydrocarbon gas through said wall and into said metal, as set forth.

7. The process of casting ingots, which consists in 15 introducing the molten metal into a mold having a wall which is permeable to gas but not to molten metal, confining a purifying gas in contact with the outer surface of said wall, and permitting the heat transferred from the molten metal to distend the pores of said wall, rarefy said 20 gas and cause it to flow through the open pores into and through said molten metal, as set forth.

8. The process of casting ingots, which consists in 25 placing an open-bottom mold upon a hollow base, confining a purifying gas in said base, pouring the molten metal into said mold, and permitting the heat transferred from said metal to that portion of the base on which said mold rests to distend the pores of said base, rarefy said 30 gas and cause a continuous flow of the gas through the open pores into and through said molten metal, as set forth.

9. The process of casting ingots, which consists in 35 placing an open-bottomed mold upon a hollow base, introducing a hydrocarbon into said base, pouring the molten metal into said mold, and permitting the heat transmitted from said metal to that portion of the base on which said mold rests to distend the pores of said base, volatilize said hydrocarbon and cause a continuous flow of reducing gas through the open pores into and through said molten metal, as set forth.

40 10. The process of casting ingots, which consists in placing an open-bottomed mold upon a porous metallic plate, arranged upon a hollow base, introducing a hydro-

carbon into said base, pouring the molten metal into said mold, and permitting the heat transmitted from said metal to said porous plate to distend the pores of said 45 plate, volatilize said hydrocarbon and cause a continuous flow of reducing gas through the open pores into and through said molten metal, as set forth.

11. The process of casting ingots, which consists in introducing a hydrocarbon into a porous but normally 50 closed hollow receptacle beneath the mold, pouring the molten metal into said mold, and permitting the heat transmitted from said metal to said receptacle to distend the pores of said receptacle, volatilize said hydrocarbon and cause a continuous flow of purifying gas 55 through its pores into the molten metal, as set forth.

12. The process of casting ingots of iron or steel, which consists in introducing the molten metal into a mold, substantially closing the upper end of said mold, delivering 60 a highly-heated purifying gas into said mold above the cast metal, and allowing the cast metal to cool, as set forth.

13. The process of casting ingots of iron or steel, which consists in introducing the molten metal into a mold, substantially closing the upper end of said mold, delivering 65 a highly-heated purifying gas into said mold above and below the cast metal, and allowing the cast metal to cool, as set forth.

14. The process of casting ingots, which consists in introducing a hydrocarbonaceous matter into a porous 70 but normally closed hollow receptacle arranged around the base of the mold, pouring the molten metal into said mold, and permitting the heat transmitted from said metal to said hydrocarbonaceous matter to volatilize said hydrocarbonaceous matter, distend the pores of said receptacle and cause a continuous flow of purifying gas 75 through its pores into the molten metal, as set forth.

In testimony, that I claim the invention set forth above I have hereunto set my hand this 30th day of January, 1900.

ADOLPHUS J. LUSTIG.

Witnesses:

FREDK. C. FRAENTZEL,  
GEO. D. RICHARDS.